

## UNITED STATES PATENT OFFICE

2,662,055

## OIL COMPOSITIONS

Charles C. Towne, Beacon, N. Y., assignor to The Texas Company, New York, N. Y., a corporation of Delaware

No Drawing. Application August 25, 1949,  
Serial No. 112,399

9 Claims. (Cl. 252—32.7)

1

This invention relates to improvements in hydrocarbon oil compositions, and more particularly to the inhibition of foam and gas entrainment in such compositions as are designed for use in special purpose oils such as are prepared for use in automatic transmission mechanisms and some types of diesel engines.

While organo-silicon oxide condensation products, including both silicones and silicates, have been indicated as foam inhibitors in lubricating oils, see Patent Nos. 2,416,503 and 2,416,504 to Trautman et al. issued February 25, 1947, they have not proven generally satisfactory in certain applications, particularly where air or gas entrainment is a problem. Air or gas entrainment is to be distinguished from so-called foam. Foam is the frothy oil and gas mixture formed on the surface of oil. It is readily distinguishable from the oil proper, the separation taking place at an oil-foam interface. Air or gas entrainment is not readily determinable and involves an actual increase in the volume of the oil because of the air or other gas entrained therein. Tests have proven that there may be gas entrainment in the absence of foam.

In the past, the efficiencies of such condensation products have been determined by their anti-foam function. Relatively simple tests have been used such as that wherein the oil to be tested is placed in a graduate and air, in the form of fine bubbles, is passed upwardly through the column of oil at a predetermined rate. The time given to form a given amount of foam may be noted or the amount of foam formed in a given time may be noted. Such a test is disclosed in the above-mentioned patents.

This test is apparently satisfactory for determining the foaming characteristics of certain types of oils for certain purposes but is not generally determinative of foaming for all types of oils and is not determinative of gas entrainment.

For example, in the development of a special purpose oil for use in hydraulic transmission mechanisms for automotive vehicles such as the General Motors Hydramatic and Dynaflow transmissions and other transmissions of the automotive type, the oil after treatment with the usual liquid dimethyl silicone polymer of 100 centistokes at a temperature of 25° C., was satisfactory as regards foaming when tested by the CRC test, the latter being a test incorporating the principle of the test disclosed in the above-mentioned patents but more extensive as regards temperatures as explained hereinafter. However,

2

when that oil was used in hydraulic transmissions, it was found to foam in substantially the same amount as if it had not been treated with the silicone polymer. Increased quantities of the polymer did not help the situation.

In the case of a lubricating oil designed for use in a particular type of diesel engine, the oil was found satisfactory by the CRC test when only small amounts of a silicone polymer of 100 cs. was used. However, in operation in the engine, the oil foamed badly and was unsatisfactory.

In both the above cases, gas entrainment as distinguished from foaming was apparently present to a large degree and appeared to be a material factor. Such gas entrainment reduces the apparent specific gravity of the oil apparently in a somewhat spotty manner so that the resultant mixture is not uniform but is characterized by random gas pockets. The transmission mechanism or the pump handling the oil becomes noisy and tends to vibrate. This is due, it is believed, to the different resistances of the oil and the oil-gas mixture or possible gas pockets alone to the mechanical mechanism. An oil with little or no gas entrainment will offer substantially uniform resistance to the mechanical mechanisms but an oil containing a considerable amount of gas dispersed at random or in pockets will vary widely in resistance. Hence, the force opposing the pump or other mechanism will vary widely and give rise to the characteristic noise and vibration. Without such gas entrainment, the oil is substantially homogeneous and exerts a uniform force against the moving elements of the mechanism.

The present invention has as its principal object the solution of the foam and gas entrainment problems in such special applications of hydrocarbon oils and the inhibition of foam and gas entrainment in the more general applications in a more efficient manner.

Another object of the invention is to provide hydrocarbon oil compositions for both general and special purposes wherein the characteristics thereof, especially foaming and gas entrainment, are greatly improved.

A further object of the invention is the provision of novel hydrocarbon oils characterized by their operation in oil-handling mechanisms in a substantially quiet and vibration-free manner.

Still another object of the invention is the provision of a method for treating hydrocarbon

oil compositions whereby undesirable gas entrainment in operation is inhibited.

Briefly stated, the present invention is based on the discovery that organo-silicon oxide condensation products of relatively high viscosities are effective in inhibiting foam and gas entrainment in hydrocarbon oils wherein like materials of relatively low viscosities are of little or no effect and are generally less efficient than the higher viscosity materials. More specifically, the invention relates to special purpose hydrocarbon oil compositions having improved foam and gas entrainment characteristics, improvement being secured by the use of organo-silicon oxide condensation products of relatively high viscosities. Such special purpose oils include hydraulic transmission oils and special oils for lubrication of diesel engines.

The organo-silicon oxide condensation products or condensation products of silanols or organo-silicols referred to herein are intended to include both silicones and silicates, preferably normally liquid, of the following general compositions:



wherein R represents similar or dissimilar organic radicals such as alkyl, aryl, alkaryl, aralkyl and heterocyclic groups; the terminal R's and OR's or other R's and OR's may be substituted by hydroxyl groups; and n is one or more. Such compounds and their methods of preparation to form compounds of different viscosities are well known to the art. Where R in the foregoing formula is an aromatic hydrocarbon grouping, intra-substituents such as a halogen, a nitrogen-containing radical as  $\text{NO}_3$  or  $\text{NH}_2$ , a sulfur-containing radical such as  $\text{SO}_3\text{H}$  or  $\text{SH}$ , or a phosphorus-containing radical such as phosphite, phosphate or the thio derivatives thereof may occur.

Typical compounds include dimethyl silicone, methyl phenyl silicone, ethyl butyl silicone, methyl cyclohexyl silicone, dicyclohexyl silicone, diphenyl silicone, hydroxy phenyl methyl silicone, phenyl propyl silicone, phenyl isopropyl silicone, tolyl butyl silicone, tolyl amyl silicone, phenyl hydroxy ethyl silicone and the corresponding polymers of methyl orthosilicate and ethyl orthosilicate. Compounds containing simple organic radicals such as methyl, ethyl and short chain alkyl groups are preferred. Such compounds may have hydroxyl groups or organic radicals as terminals.

The compounds are preferably incorporated in the composition to be treated by mixing them with a high boiling naphtha such as kerosine and mixing the resultant combination with the composition. For the purpose of the following description, it will be understood that sufficient kerosine is added to 10 grams of the specific silicone or similar compound to make up a total of 100 ml.

Before proceeding to a detailed description of the invention, the various tests used for determining the foaming characteristics of hydrocarbon oils should be reviewed.

In the so-called CRC test, oil in a graduate is heated to  $120^\circ \text{ F.}$  and cooled to  $75^\circ \pm 5^\circ \text{ F.}$

In sequence 1, air at a rate of 0.2 cubic feet per hour is bubbled through the oil through a diffusion plate at the bottom of the graduate. The foam height is recorded at the end of a five minute period, thus giving the zero minute reading. The air is shut off and the foam is recorded again at the end of a ten minute period, thus giving the ten minute reading. In sequence 2, the same steps are followed except that the temperature is raised to  $200^\circ \pm 5^\circ \text{ F.}$  In sequence 3, the same steps are repeated with the temperature returned to  $75^\circ \pm 5^\circ \text{ F.}$

In the Carnegie foam test which has been developed primarily for the testing of oils used in hydraulic transmission mechanisms and the like, the oil being tested passes through a pump having a submerged intake and an air-open discharge above the body of oil. Simultaneously two propellers are used to agitate the oil body. The oil is heated to a temperature of about  $200^\circ \text{ F.}$

After the oil is brought to temperature, the propeller motor is turned on and the pump discharge pressure set at 40 lbs. per square inch. After one minute, the motor is shut off and the height of foam, i. e., the distance from the top of the foam to the oil-foam interface, is measured. The foam collapse time is taken as the time elapsing between the stopping of the motor and the first appearances of the oil surface through the foam. The foam height is reported to  $\frac{1}{8}''$  and the foam collapse time to one second. Approximately six quarts of oil are required for the test.

The VVL test is based on a proposed Federal specification of October 4, 1941, for universal gear lubricants. It involves the churning of the lubricant in a Mixmaster or its equivalent having a pan 7" in diameter and  $3\frac{1}{4}$ " deep, the pan being supported on the turn-table mounted in the center bearing hole of the two bearing holes in the Mixmaster base plate. 500 ml. of the lubricant is churned with concave paddles at room temperature for 15 minutes at a beater speed of 550 R. P. M. After the churning period, the lubricant is allowed to stand one hour. The foam is measured at zero minutes and at ten minute intervals through one hour.

In the Towne foam test, a Mixmaster or the equivalent is used in combination with a 500 ml. graduate cylinder. 400 grams of the sample is heated to  $150^\circ \text{ F.}$  and maintained at that temperature for 30 minutes. It is then allowed to cool to room temperature by standing for a sufficiently long period. 200 grams of the test oil is weighed into an 800 ml. beaker and placed in a constant temperature bath at the test temperature of  $75^\circ \text{ F.}$  After reaching temperature, the oil is stirred for exactly three minutes. The contents of the beaker are then poured quickly into a 500 ml. graduate cylinder and the graduate placed in the temperature bath. The volume of foam is determined at 0, 10, 20, 30, 40, 50 and 60 minutes starting with zero time as four minutes after the stirring operation is begun. In this test, the oils of SAE 10, 20 and 30 grades are tested at  $75^\circ \text{ F.}$  and oils of SAE 40, 50 and 60 grades are tested at  $120^\circ \text{ F.}$

In all the foregoing tests, the objective has been to measure the foam and no attention has been paid to gas entrainment. Apparently gas entrainment and its possible effect in use of the oil has been entirely overlooked.

As an example of a practical application of the invention, a hydraulic transmission fluid was prepared with a mineral oil base. About 3.5 to

5

4.5% of an additive of the methacrylate polymer type, about 2.5 to 3.5% of an additive of the sulfurized sperm oil type and about 0.8 to 1.0% of an additive of a barium thiophosphate-sodium sulfonate type in a light oil as a carrier, all by weight, were added to a base compound formed of a refined paraffin base oil having a viscosity SSU at 100° F. of about 100.

The methacrylate polymer type additive contains approximately 40% of a polymerized ester of methacrylic acid having a molecular weight between 10,000 and 15,000 and of the following general formula:



wherein R is a mixture of alkyl groups having from 8 to 16 carbon atoms such as cetyl, lauryl and octyl groups. The additive is formed by dissolving the polymer in a Mid-Continent solvent-refined 150 neutral oil. The result is a clear, light-amber colored viscous fluid having a Sp. Gr. 60°/60° F. of 0.89-0.90, and flash point °F., diluted to 10% solids with a S. A. E. 20 oil, COC, of 405 min., a viscosity, Kinematic at 210° F., cs. of 600-800 and a Neut. No. of 0.4 max. This additive has been found valuable as a viscosity index improver and a pour point depressant.

The sulfurized sperm oil type additive can be described as having a sulfurized sperm oil and lanolin base, the principal constituent being a sulfurized derivative of cetyl oleate:



It is probable that the sulfur enters the molecule at the double bond to form a ring structure somewhat as follows:



The additive has a gravity °API of 14.5-16.0; a viscosity S. U. S. at 210° F. of 190 to 230 seconds, and a saponification number of 140-155. The sulfur content is about 9 to 11% by weight. In addition to functioning as an extreme pressure lubricant, the additive also functions as an oxidation inhibitor and as a mild detergent.

The barium thiophosphate-sodium sulfonate type additive is formed of approximately 12% sodium sulfonate, about 45.5% light lubricating oil as a carrier and about 42.5% of a barium compound of the following type:



wherein R=C<sub>7</sub>+C<sub>8</sub>+C<sub>10</sub> alcohols. The additive is a dark oily liquid of a density of about 1.016. It contains about 6.0 to 7.3% barium, about 2.6 to 3.2% phosphorus, about 6.0 to 7.9% sulfur, and about 0.25 to 0.40% sodium all by weight. Its principal function is as an antioxidant.

With the addition of 225 parts per million of 100 cs. silicone (dimethyl silicone polymers) in kerosine (about 22.5 p. p. m. silicone) to the above-described hydraulic transmission fluid, a Carnegie foam test of the fluid showed a foam height of  $\frac{1}{2}$ " and a foam collapse time of 42 seconds. When only 100 p. p. m. of the same silicone but of 1,000 cs. in kerosine (about 10 p. p. m. silicone) was used, the foam height was less than

6

1/8" and the foam collapse time was zero, that is, there was no sustained foam. The use of the higher viscosity silicone also appeared to substantially inhibit gas entrainment since the oil so treated when used in a transmission enabled quiet and smooth operation in contrast to the noisy operation when oil treated with the silicone of 100 cs. was used. This particular fluid had a viscosity SSU at 100° F. of 204.4 and at 210° F. of 52.3. It had a viscosity index of about 140.

about 110.

A comparison of the 22.5 p. p. m. 100 cs. silicone giving a foam height of  $\frac{1}{2}$ " and the 10 p. p. m. 1,000 cs. silicone giving a foam height of less than  $\frac{1}{8}$ " establishes the 1,000 cs. silicone as being far more efficient than a silicone of the same composition but of lower viscosity. In brief, the 1,000 cs. material when used in an amount less than 45% of the 100 cs. material was 15 four times as effective in inhibiting foam. 20

On a further test of this same fluid at temperatures ranging from 200° to 275° F. with silicone (1,000 cs.) contents of 10-15 p. p. m., the foam height was  $\frac{1}{4}$ " or less and the foam collapse time except at extremely high temperatures was zero. At the high temperature of 275° F., the foam required only 23 seconds for collapse.

This particular fluid is a particularly good hydraulic transmission fluid in that it is capable of transmitting power efficiency through either the fluid coupling or torque converter, it is an efficient lubricant for the complicated and precisely machined moving parts such as the various pump units involved, and is capable of satisfactorily lubricating and preventing wear on any gearing contained in the transmission unit. It has the correct viscosity and a pour point of at least  $-35^{\circ}$  F. which satisfies the requirements of temperature extremes liable to be encountered. It is stable in service, resistant to oxidation and deposit formation, and resistant to foam formation and gas entrainment which could interfere with the efficiency of the power transmission.

45 Strange to say, the increased efficiency of the  
higher viscosity silicone in this particular fluid is  
not indicated by the CRC or similar tests that  
determine only foam presumably because such  
tests do not simulate the actual operation in a  
50 hydraulic transmission and do not determine gas  
entrapment.

Respecting this particular hydraulic transmission fluid, it has been found that regardless of the amount of 100 cs. silicone employed, the foam as determined by the Carnegie foam test cannot be reduced sufficiently to pass specifications. On the other hand, the use of silicones of higher viscosities has solved the foam problem.

In another instance, a special lubricating oil was prepared for use in diesel engines by combining a base oil (having a gravity, API of 22.5-28.5, flash, C. O. C. min. 420° F., fire, C. O. C., min. 470° F., viscosity, S. S. U. at 100° F. of 540-630, viscosity index 76 min., pour point 5° F. max.) with about 16.5% by volume of an additive classified as a basic barium sulfonate, barium dithiophosphate, sulfurized terpene product, the latter being particularly valuable in counteracting the corrosive effects of high sulfur fuels.

70 When tested by the CRC foam test, the addition of a dimethyl silicone polymer of 100 cs. in amounts up to 20 p. p. m. was of very little value in reducing the initial foam height. For instance, with 2.5 p. p. m. silicone, the foam at 5  
75 minutes was 310 ml. When an equivalent

amount of the same silicone of 1,000 cs. was used, the foam at 5 minutes was only 150 ml., a reduction of about 52%. With 5 p. p. m. of the silicone of 100 cs. 300 ml. foam was obtained in 5 minutes. An equivalent amount of 1,000 cs. silicone of the same composition reduced the foam at 5 minutes to 50 ml., a reduction of about 83%.

With 10 p. p. m. of the 100 cs. silicone, 250 ml. foam was produced in 5 minutes. With an equivalent amount of 1,000 cs. silicone, only 30 ml. foam was formed at 5 minutes, a reduction of about 88%. Even with 100 p. p. m. of the 100 cs. material, 70 ml. foam was formed in 5 minutes.

In connection with the relation of gas entrainment, its ill-effects and its determination, tests were run with a straight naphthene base oil having a gravity ° API of 18.0 to 21.0, flash, COC ° F. min., 370, fire, COC ° F. min., 420, viscosity, S. S. U. at 100° F. of 550-580, viscosity S. S. U. at 210° F. of 53-56 neutralization number of 0.1 max., and with no additives of any type contained therein. In this case, both in actual operation and in laboratory tests, the higher viscosity organo-silicon compounds were found effective as regards the inhibition of both foaming and gas entrainment whereas the lower viscosity compounds were found to be of little or no effect. This particular oil is of special value in the lubrication of large diesel engines such as those of Nordberg manufacture (model TS-2 cycle).

In one specific instance, the installation included six Nordberg 2-cycle diesel engines of 7325 horsepower rating each with generators directly connected thereto. In this installation each engine had a gear train comprising four large gears with an oil spray at each gear meshing. When operating with straight oil, there was a great deal of rattling and vibration in the circulating pumps for this oil, apparently due to air (or fixed gas) entrained in the oil by the aforesaid gear trains.

With the addition of a dimethyl silicone of 100 cs. in an amount equivalent to about 3 p. p. m., there was no noticeable change in the noise or vibration of the pumps. With the use of about 3 to 4 p. p. m. of the same silicone but of 1,000 cs., there was immediate and substantially permanent improvement in that the noise and vibration were substantially eliminated.

To check the effect of the higher viscosity silicones, the operation of the engine insofar as the oil is concerned was simulated in the laboratory by the use of a circulating unit formed of standard pipe and fittings where the oil was circulated by a Chevrolet automobile water pump driven by a  $\frac{1}{4}$  H. P. motor at a speed of about 2100 R. P. M. Air was added to the system at the suction side of the pump and the circulating oil heated by a thermostatically-controlled electric heater. In this way, the actual conditions in the engine as to the entrainment of air and temperature were simulated. The unit was charged with 5000 cc. oil and the oil circulated at 130° F. with 40-60 cc./min. of air being added to the suction side of the pump. Both the foam height and increase of volume of oil due to air entrainment were determined by observing levels in a sight glass on the top of the unit.

When the simulated engine test unit was conducted with 275 cc. straight oil, the volume of the oil increased to 310 cc., an increase of about 13%. Additionally there was about 20 cc. foam. The addition of dimethyl silicone of 100 cs. in amounts of 3, 6, 25 and 50 p. p. m. gave only a slight reduction in the air entrainment, i. e., the

volume increase of the oil was reduced to about 8%. Foam was still formed.

With a fresh charge of oil, a dimethyl silicone of 1,000 cs. was used in amounts of 5, 10, 50 and 100 p. p. m. The 5 and 10 p. p. m. additions were found to reduce the volume increase of the oil and the 50 p. p. m. addition substantially eliminated all volume increase. Increased amounts of silicone did not have any adverse effect. This particular test was continued for more than two days during which time there was no change in the volume of oil.

Another run was made with the same silicone but of 100,000 cs. in a concentration of about 5 p. p. m., the silicone being dissolved or dispersed in ethyltriethoxy silane. With a concentration of 5 p. p. m. corresponding to about 40 p. p. m. of the silane, there was some reduction in air entrainment or volume increase. With a second 5 p. p. m. addition, making a total of 10 p. p. m., the air entrainment was reduced to substantially zero. The silicone was effective over the three days of the test.

The apparatus was thoroughly cleaned between each test.

It should be added that silicones of 500 cs. were tried in the same oil with the more conventional foam tests. About 7% foam was produced and special measurements of the increase in volume of the oil showed an increase of about 7%.

Summarizing this experience, it will be noted that with this oil having a tendency to increase in volume up to 13%, the silicones of 100 cs. and 500 cs. were substantially ineffective whereas silicones of 1,000 cs. and 100,000 cs. were substantially and completely effective. These results are particularly significant since they demonstrate the value of the simulated engine test in determining both foam and gas entrainment and illustrate the efficiency of the higher viscosity silicones in a straight oil in which there are no oil improving additives or agents of any type and in which foaming and gas entrainment are problems.

Equivalent increased efficiencies of organo-silicon compounds of higher viscosities have been demonstrated in tests with other types of hydrocarbon oils.

In test on a typical base oil, dimethyl silicones of low viscosities such as 6.2 cp. (about 6.4 cs.) and 85 cp. (about 87 cs.) were found in the CRC foam test, sequence 1, to hold the foam down to 10 ml. after 5 minutes whereas dimethyl silicone of 884 cp. (about 910 cs.) in the same proportion was found to prevent any foaming whatsoever.

In the case of an industrial gear lubricant having a viscosity SSU at 100° F. of 2250-2450, the base lubricant when tested as to foam characteristics by the VVL foam test, gave 500 ml. foam at the 0, 15, 30 and 45 minute intervals and 450 ml. at the 60 minute interval.

With the addition of 5 p. p. m. of dimethyl silicone of 1,000 cs., the foam at zero minutes was only 50 ml. and the foam at the remaining intervals was only 25 ml. When 1.4 p. p. m. of dimethyl silicone of 250,000 cs. was used, 50 ml. of foam was obtained at the zero and 15 minute intervals, 25 ml. at the 30 minute intervals, and only traces of foam at the 45 and 60 minute intervals.

The results of such tests indicate even greater effectiveness of the organic-silicon compounds of higher viscosities.

In the case of a refrigerator oil having a viscosity SSU at 100° F. of 300-324 and containing

an additive of the methacrylate polymer type, the oil was tested according to the Towne foam test and showed 300 ml. of foam at 0 minutes and 0 ml. in 10 minutes. The addition of 2.5 p. p. m. dimethyl silicone of 1,000 cs. reduced the 0 minute foam to 10 ml., a reduction of about 97% and the 10 minute foam to 0, a reduction of 100%. The same results were obtained with the use of only 1.4 p. p. m. or approximately one-half as much dimethyl silicone of 50,000 cs.

With a rock drill lubricant having a viscosity SSU at 100° F. of 550-610, tested by the CRC foam test, sequence 1, the foam at 0 minutes was 540 ml. and the foam at 10 minutes was 440 ml. In sequence 2, the foam at 0 minute was 160 ml. and at 10 minutes was 0. In sequence 3, the foam at 0 minutes was 690 ml. and at 10 minutes was 620 ml. The addition of 1 p. p. m. of dimethyl silicone of 100 cs. showed very little improvement as respects sequences 1 and 2, the foam at 0 minutes in sequence 3 being reduced to 100 ml.

The use of an equivalent amount of dimethyl silicone of 1,000 cs. reduced the foam in sequence 1 to 30 ml. at 0 minutes, a reduction of 94% and to 0 at 10 minutes, a reduction of 100%. In sequence 2, the foam at 0 minutes was 80 ml., a reduction of 5% and 0 at 10 minutes, a reduction of 100%. In sequence 3, the foam at 0 minutes was 20 ml., a reduction of 97% and at 10 minutes was 0, a reduction of 100%. Substantially the same results were obtained by the use of only 0.8 p. p. m. of a silicone of 10,000 cs., with 0.5 p. p. m. of a silicone of 50,000 cs., with 0.4 p. p. m. of a silicone of 100,000 cs., and with 0.3 p. p. m. of a silicone of 250,000 cs.

In a Carnegie foam test on an oil formed from a base oil and an additive of the methacrylate polymer type and having a viscosity SSU at 100° F. of about 198, the oil with 7 p. p. m. dimethyl silicone of 100 cs. had a foam height of  $\frac{1}{8}$ " and a foam collapse time of 39 seconds. When treated with only 5 p. p. m. of the same type silicone of 1,000 cs., the foam height was less than  $\frac{1}{8}$ " and the foam collapse of the order of 25 seconds.

The same oil treated with 10 p. p. m. of silicone of 100 cs. showed a foam height of  $\frac{1}{4}$ " and a foam collapse time of 39 seconds. When treated with 10 p. p. m. of a like silicone of 1,000 cs., the foam height was less than  $\frac{1}{8}$ " and the foam collapse time was 0, i. e., there was no continuous layer of foam.

The same base oil treated with 80 p. p. m. of 100 cs. silicone had a foam height of  $\frac{1}{8}$ " and a foam collapse time of 20 seconds, thus, indicating the improved anti-foam efficiency of the higher viscosity organo-silicon compound.

The improved results in inhibition of foam and gas entrainment obtained by the higher viscosity organo-silicon compounds is evidenced by their proven greater efficiency even when used in smaller quantities and their ability to inhibit foam and gas entrainment in some instances where the low viscosity materials are substantially ineffective. This is particularly true in uses such as in hydraulic transmissions and in some pumps wherein the oil is subjected to turbulence in the presence of air or some other gas.

From the data obtained thus far, the effective higher viscosity organo-silicon compounds range from viscosities SSU 25° C. of about 900 cs. to 250,000 cs., and there is reason to conclude that the compounds are increasingly effective in proportion to their viscosities.

While the invention has been described in connection with hydrocarbon oil compositions, it is to be understood that it is also applicable to other organic liquids and mixtures containing the same.

Obviously many modifications and variations of the invention as above set forth may be made without departing from the spirit and scope thereof, and, therefore, only such limitations should be imposed as are indicated in the appended claims.

I claim:

1. A substantially non-foaming and non-gas entraining composition of matter comprising a major portion of a liquid hydrocarbon oil and a minor proportion of an additive and a liquid dihydrocarbon silicone polymer of a minimum viscosity of about 900 cs.

2. A power transmitting fluid for use in hydraulic transmissions and the like comprising hydrocarbon oil, an additive containing a methacrylate polymer having a molecular weight of between 10,000 and 15,000, an additive of the sulfurized sperm oil type, an additive of the barium thiophosphate-sodium sulfonate type, and sufficient of a liquid dihydrocarbon silicone of a minimum viscosity of about 900 cs. to inhibit foaming and gas entrainment thereof in operation.

3. A power transmitting fluid for use in hydraulic transmissions and the like comprising hydrocarbon oil, about 3.5 to 4.5% of an additive containing a methacrylate polymer having a molecular weight of between 10,000 and 15,000, about 2.5 to 3.5% of an additive of the sulfurized sperm oil type, about 0.8 to 1.0% of an additive of the barium thiophosphate-sodium sulfonate type, all by weight, and sufficient of a liquid dihydrocarbon silicone of a minimum viscosity of about 900 cs. to inhibit foaming and gas entrainment thereof in operation.

4. A power transmitting fluid for use in hydraulic transmissions and the like consisting essentially of hydrocarbon oil, about 3.5 to 4.5% by weight of an additive consisting essentially of about 40% by weight of a polymerized ester of methacrylic acid having a molecular weight between 10,000 and 15,000 and of the following general formula:



5. Wherein R is a mixture of alkyl groups having from 8 to 16 carbon atoms, about 2.5 to 3.5% by weight of an additive comprising lanolin and a sulfurized derivative of cetyl oleate, about 0.8 to 1.0% by weight of an additive comprising sodium sulfonate and a barium compound of the following general formula:



6. Wherein R =  $\text{C}_7+\text{C}_8+\text{C}_{10}$  alcohols, and sufficient of a liquid dihydrocarbon silicone of a minimum viscosity of about 900 cs. to inhibit foaming and gas entrainment of the fluid in operation.

7. A power transmitting fluid for use in hydraulic transmissions and the like comprising a refined paraffin base hydrocarbon oil having a viscosity of about 100 SSU at 100° F., about 3.5 to 4.5% by weight of an additive comprising about 40% by weight of a polymerized ester of

## 11

methacrylic acid having a molecular weight between 10,000 and 15,000 and of the following general formula:



wherein R is a mixture of cetyl, lauryl and octyl groups, about 2.5 to 3.5% by weight of an additive comprising lanolin and a sulfurized derivative of cetyl oleate, about 0.8 to 1.0% by weight of an additive comprising about 12% by weight sodium sulfonate and about 42.5% by weight of a barium compound of the following general formula:



wherein R=C<sub>7</sub>+C<sub>8</sub>+C<sub>10</sub> alcohols, and sufficient of a liquid dimethyl silicone of a minimum viscosity of about 900 cs. to inhibit foaming and gas entrainment by the fluid in operation.

6. A power transmitting fluid for use in hydraulic transmissions and the like comprising a refined paraffin base hydrocarbon oil having a viscosity of about 100 SSU at 100° F., about 3.5 to 4.5% by weight of an additive comprising about 40% by weight of a polymerized ester of methacrylic acid having a molecular weight between 10,000 and 15,000 and of the following general formula:



wherein R is a mixture of cetyl, lauryl and octyl groups, about 2.5 to 3.5% by weight of an additive comprising lanolin and a sulfurized derivative of cetyl oleate, about 0.8% to 1.0% by weight of an additive comprising about 12% by weight sodium sulfonate and about 42.5% by weight of a barium compound of the following general formula:



## 12

wherein R=C<sub>7</sub>+C<sub>8</sub>+C<sub>10</sub> alcohols, and sufficient of a liquid dimethyl silicone of a viscosity of about 1,000 cs. to inhibit foaming and gas entrainment by the fluid in operation.

- 5 7. A composition of matter consisting essentially of a liquid hydrocarbon and an additive, and sufficient of a liquid dimethyl silicone polymer of a viscosity of about 1,000 cs. to inhibit foaming and gas entrainment.
- 10 8. A lubricating composition adapted for use as a diesel lubricant with fuels of relatively high sulfur content comprising a liquid hydrocarbon and a substantial proportion of an additive consisting essentially of basic barium sulfonate, barium dithiophosphate and a sulfurized terpene, and sufficient of a liquid dihydrocarbon silicone of a minimum viscosity of about 900 cs. to inhibit foaming and gas entrainment in operation.
- 15 9. A lubricating composition adapted for use as a diesel lubricant with fuels of relatively high sulfur content comprising a hydrocarbon oil having a C. O. C. flash point of about 420° F. and a viscosity of 540-630 SSU at 100° F., about 16.5% of an additive consisting essentially of basic barium sulfonate, barium dithiophosphate and a sulfurized terpene, and sufficient of a liquid dihydrocarbon silicone of a viscosity of about 1,000 cs. to inhibit foaming and gas entrainment in operation.
- 20 30 CHARLES C. TOWNE.

## References Cited in the file of this patent

## UNITED STATES PATENTS

| Number    | Name          | Date          |
|-----------|---------------|---------------|
| 2,375,007 | Larsen et al. | May 1, 1945   |
| 2,438,446 | Leland        | Mar. 23, 1948 |
| 2,439,281 | Foehr         | Nov. 29, 1949 |
| 2,533,700 | Wallace       | Dec. 12, 1950 |
| 2,589,317 | Young et al.  | Mar. 18, 1952 |

## OTHER REFERENCES

Kauppi et al., "Organic-Silicon Compounds for Insulating Electrical Machines," Reprinted from Transactions of the American Institute of Electrical Engineers, N. Y. C., N. Y., vol. 64, 1945, 4 pages.

50 Kauppi et al., "Silicone Fluids in Hydraulics and Lubrication," Reprinted from Product Engineering, February 1949, 5 pages.